

# United States Patent Office

2,917,461

Patented Dec. 15, 1959

1

2,917,461

## FERROMAGNETIC MATERIAL AND METHOD OF PREPARATION THEREOF

Lothar Heinrich Brixner, Wilmington, Del., assignor to E. I. du Pont de Nemours and Company, Wilmington, Del., a corporation of Delaware

No Drawing. Application June 14, 1957  
Serial No. 665,632

4 Claims. (Cl. 252—62.5)

This invention relates to a new ferromagnetic material and more particularly to a strontium-aluminum-ferrate.

Ferromagnetic materials might broadly be classified into two groups: those with low coercivities, and those with high coercivities. Materials of the former type are useful in transformers, magnetic amplifiers, memory cores, and microwave devices, and include such well-known substances as the Permalloys, silicon irons, and certain ferrites—the ferrites being materials having the general formula  $MO \cdot Fe_2O_3$  where M is a divalent metal. The ferromagnetic materials with high coercivities include the permanent magnetic materials, such as  $BaO \cdot 6Fe_2O_3$ , and manganese bismuthide (MnBi). It follows, obviously, that ferromagnetic materials of high coercivity provide better permanent magnet characteristics than those with low coercivity. The ferromagnetic material described in this invention possesses an exceptionally high intrinsic coercive force, and it is represented by the chemical formula  $SrAlFeO_4$ . It has a crystalline structure, but this structure is unlike that of such known ferromagnetic materials as the ferrites and  $BaO \cdot 6Fe_2O_3$ .

The composition of this invention may be prepared by presintering a finely divided mixture of aluminum oxide, strontium carbonate and ferric oxide. The presintered product is cooled and ground to a powder and then compacted into a unitary mass of desired shape by pressing or extruding. The shaped product is then fired at temperatures above about 900° C.

For a clearer understanding of the invention, the following specific example is given. This example is intended to be merely illustrative of the invention and not in limitation thereof. Unless otherwise specified all parts are by weight.

### Example

According to the equation:



stoichiometric quantities of the reactants (0.6804 part by weight  $Fe_2O_3$ , 0.4353 part by weight  $Al_2O_3$  and 1.2580 parts by weight  $SrCO_3$ ) were carefully mixed and finely ground together in an agate mortar to a fineness of —200 mesh. After thorough mixing, the powder was placed in a platinum crucible and heated in air to 800° C. for 6 hours, after which the crucible was taken from the furnace and the reaction product cooled in the crucible to room temperature. The product at this point was a dark brown material which turned olive brown upon grinding to small particle size. A portion of the product was tested with hydrochloric acid for the presence of carbonate and found to be carbonate-free. The material was again ground in an agate mortar to —200 mesh, and the powdered product was pressed into a button  $\frac{1}{2}$  inch in diameter under a pressure of 40,000 p.s.i. This button was fired at 1200° C. in air for 8 hours, and cooled. The product obtained was dark brown, and it was useful as a magnet. X-ray analysis showed that it was crystal-

2

line in structure, and that it contained none of the original components.

The material thus prepared was found to have the following magnetic properties:

5 Saturation magnetization,  $B_s$  gauss 13  
Magnetic moment/gram,  $\sigma_s$  ergs/gauss 0.56  
Intrinsic coercive force,  $iH_c$  oersteds 970  
Resistivity ohm cm  $5 \times 10^7$

10 The above value for intrinsic coercive force was obtained when the compound was magnetized in an external field of 2900 oersteds, which proved to be not high enough to saturate the compound. When a magnetizing field of 5500 oersteds was used, the  $iH_c$  was 2028 oersteds. These results indicated that the compound should be magnetized in a field of 7000 to 10,000 oersteds to be saturated.

15 The above values of the magnetic properties were obtained on a pulverized sample having an apparent density of 1.90 gms./cc.

20 Measurements were made in the following manner. The sample is placed in one of two coils which are matched inductively, and are connected in series opposition with one another, and are in series with a set of variable resistances and a ballistic gal-

25 vanometer. The test coils are placed inside of a solenoid in such a manner that both are in fields at equal magnitude. A change in the solenoid field causes a corresponding change in the magnetization of the sample which induces a proportional current in the test coil and

30 galvanometer circuit. Calibration against a specimen of known properties permits the measurement of the properties of new materials.

35 Alternatively, other decomposable compounds might be used as starting materials to produce  $SrAlFeO_4$ .

Among these would be  $Sr(OH)_2$ ,  $Sr(NO_3)_2$ ,  $Fe(NO_3)_3$ ,  $Al(OH)_3$  or  $Al(NO_3)_3$ . The choice of starting material would be dependent on the purity in which it could be obtained and its cost. Commercially available products of the highest purity are preferred. Although I have

40 chosen to presinter my crystalline material at 800° C. for a period of 6 hours, any temperature between 600° C. and 1000° C. may be used, with time of heating from 4 to 10 hours. Similarly, although the second firing of

45 my crystalline material was carried out at 1200° C. for 8 hours, the temperature for this firing may be from 900° C. to 1400° C. with the time of heating being between 6 and 10 hours.

50 One of the outstanding advantages offered by the product of this invention is that it can be used to make powerful magnets possessing great resistance to demagnetizing fields, and of minimum size and weight. These magnets may be used in rotating mechanical couplings, television focusing yokes, refrigerator and cabinet door latches, motors and generators.

55 Since it is obvious that many changes and modifications can be made in the above-described details without departing from the nature and spirit of the invention, it is to be understood that the invention is not to be limited to said details except as set forth in the appended claims.

60 I claim:

1. As a new composition of matter, a ferromagnetic material of the chemical formula  $SrAlFeO_4$ .

2. A process for preparing a ferromagnetic material which comprises presintering by heating at a temperature from about 600° C.—1000° C. for about 4—10 hours a mixture comprising (1) an inorganic strontium compound selected from the group consisting of  $Sr(OH)_2$ ,  $Sr(NO_3)_2$  and  $SrCO_3$ , (2) an inorganic aluminum compound selected from the group consisting of  $Al(OH)_3$ ,  $Al_2O_3$ , and  $Al(NO_3)_3$ , and (3) an inorganic iron compound selected from the group consisting of  $Fe(NO_3)_3$  and  $Fe_2O_3$ , said strontium, aluminum and iron compounds being present

in the mixture in stoichiometric amounts based on the formation of  $\text{SrAlFeO}_4$ , cooling the presintered product thus obtained, grinding the product to a powder, compacting the powder into a unitary mass and heating said mass at a temperature ranging between  $900^\circ\text{ C.}-1400^\circ\text{ C.}$  for from 6-10 hours and recovering a ferromagnetic material.

3. A process for preparing a ferromagnetic material which comprises presintering by heating at a temperature from about  $600^\circ\text{ C.}-1000^\circ\text{ C.}$  for about 4-10 hours a mixture comprising  $\text{SrCO}_3$ ,  $\text{Al}_2\text{O}_3$ , and  $\text{Fe}_2\text{O}_3$ , said strontium, aluminum and iron compounds being present in the mixture in stoichiometric amounts based on the formation of  $\text{SrAlFeO}_4$ , cooling the presintered product thus obtained, grinding the product to a powder, compacting the powder into a unitary mass and heating said mass at a temperature ranging between  $900^\circ\text{ C.}-1400^\circ\text{ C.}$  for from 6-10 hours and recovering a ferromagnetic material.

4. A process for preparing a ferromagnetic material which comprises presintering by heating at a temperature

of about  $800^\circ\text{ C.}$  for about 6 hours a mixture comprising  $\text{SrCO}_3$ ,  $\text{Al}_2\text{O}_3$ , and  $\text{Fe}_2\text{O}_3$ , said strontium, aluminum and iron compounds being present in the mixture in stoichiometric amounts based on the formation of  $\text{SrAlFeO}_4$ , cooling the presintered product thus obtained, grinding the product to a powder, compacting the powder into a unitary mass and heating said mass at a temperature of about  $1200^\circ\text{ C.}$  for about 8 hours, and recovering a ferromagnetic material.

References Cited in the file of this patent

Adelskold: Askiv for Kemi, Mineralogi Och Geologi, Band 12A, pp. 8 and 9 (1938).

Jonker et al.: Physica, XVI, p. 340, March 1950.

Kordes et al.: Chemical Abstracts, vol. 46, col. 4411, May 25, 1952.

Gorter: Philips Research Reports, vol. 9, pp. 403, 404, 428, 432, December 1954.

Fresh: Proceedings of Inst. Radio Eng., October 1956, pp. 1303-13.